

C. S. BRADLEY,  
PRODUCTION OF IRON AND STEEL,  
APPLICATION FILED OCT. 5, 1916.

1,353,716.

Patented Sept. 21, 1920.



INVENTOR  
Charles S. Bradley  
BY  
Knight, *Knight*  
ATTORNEYS

# UNITED STATES PATENT OFFICE.

CHARLES S. BRADLEY, OF NEW YORK, N. Y.

## PRODUCTION OF IRON AND STEEL.

1,353,716.

Specification of Letters Patent. Patented Sept. 21, 1920.

Application filed October 5, 1916. Serial No. 123,873.

To all whom it may concern:

Be it known that I, CHARLES S. BRADLEY, a citizen of the United States, residing in the city, county, and State of New York, have 5 invented certain new and useful Improvements in the Production of Iron and Steel, of which the following is a specification.

My invention relates to the production of metals, such as for example iron and steel, 10 from metal bearing substances.

The principles of the invention will be clearly understood from the description of a specific embodiment thereof for the production of iron from the ore.

15 One of the important features of the invention is to produce a non-coherent mixture of finely divided metal and gangue and to separate the metal from the gangue without resorting to the operation of slagging the 20 aluminous and silicaceous material. Another important feature of the invention resides in the reduction of the metal content of the ore or other metal bearing substance to metallic form at a temperature below the fusion 25 point of the metal. A further feature of importance is an improved process and apparatus for the separation of the finely divided metal from the gangue material.

30 Apparatus suitable for carrying out the process is diagrammatically shown in the accompanying drawing.

In said drawing:

Figure 1 represents a system for the treatment of finely crushed ore, comprising 35 reduction and separation apparatus, with one form of apparatus for consolidating the separated metal after its removal from the gangue; and

40 Fig. 2 represents another embodiment of the consolidating apparatus, wherein the finely divided material is made coherent by pressure.

It is assumed in the example of the invention which will be described, that iron ore, 45 for example in the form of oxid or carbonate, has already been finely crushed and dried, before being subjected to the treatments herein described.

50 Referring in detail to the annexed drawing, 10 indicates a reduction drum to which the finely crushed and dried iron ore is fed by way of the hopper 11 and screw conveyer 12. The drum 10 is mounted on suitable bearing rollers 13, one or more of which may 55 be suitably driven to effect a rotation of the drum. A series of longitudinal riffles or ribs

14 raise the crushed ore which repeatedly falls from the top of the drum through a heated reducing gas which is maintained within the drum, as will be described. A 60 spiral discharge 15 conveys the reduced mixture in finely divided non-coherent form to the discharge neck 16 from which it is delivered by the chute 17 to a conveyer belt 18. The reduced ore on its way to the conveyer belt 18 is subjected to the influence of a magnet 19 of metal construction, which attracts the finely divided metal particles and magnetically conveys them to a point above the metal discharge hopper 20. The 65 gangue from which the metal has thus been removed is delivered by the conveyer belt 18 to a gangue hopper 21 from which it is discharged in any suitable manner as for example by the screw conveyer 22. The metal 70 hopper 20 has its discharge neck submerged within the body of molten metal maintained within the crucible 23 which is suitably heated, as for example by means of the gas flame 24.

80 The electro-magnet 19 forms a roof over the separating chamber and comprises a suitably formed body of iron or the like having perforations 25 for the reception of water cooling pipes 26 through which the 85 magnet coils or windings are led for producing the magnetic flux employed in the separation of the finely divided metal from the gangue. The magnet windings are supplied with multiphase alternating current 90 and suitably connected to produce a progressive magnetic pole or series of poles which advance from left to right in the drawing. I have illustrated the connections for three phase alternating current, merely 95 by way of example. These windings may be connected in star connection at the discharge end and likewise the separate water cooling pipes may be united with a common discharge pipe at the end. An air pipe 27 may 100 be employed to deliver air into the discharge end of the drum 10 and a gas pipe 28 may lead a reducing gas such as natural gas into the separation chamber, the current of the air and gas being from right to left in the 105 drawing, resulting in the production of a flame in the discharge end of drum 10 whereby the reducing temperature is maintained. The reducing gas supplied through pipe 28 will represent in proportion to the 110 air delivered through pipe 27, that quantity which will not only maintain the reduc-

110

ing temperature, but will also provide the necessary amount of reducing agent for the metal content of the ore. In the case of ore containing ferric oxide  $Fe_2O_3$  being reduced 5 to metallic iron by the action of natural gas,  $CH_4$ , the temperature would be maintained at a low red heat and the chemical reaction might be represented by the equations



An excess of gas is necessary on account 10 of the equilibrium constants of the products of reaction. The products of combustion 15 and reduction gas are discharged from the drum 10 into the flue 29.

I have shown in Fig. 1, a metal consolidating apparatus which operates on the principle of fusion. In Fig. 2 the consolidating apparatus comprises an extrusion or squirming nozzle or die 30 which receives the finely divided metal from the metal hopper 20 and in which the finely divided metal is subjected to compression by the hydraulic 25 plunger 31 under suitable control. A spring 32 returns the plunger to normal position within its cylinder 33 and the hydraulic fluid is admitted by way of the port 34 to reciprocate the plunger in the compressing 30 or consolidating operation. With each stroke of the plunger, a corresponding discharge of consolidated metal occurs from the outlet of the die 30, which product may be severed into unit lengths in any suitable 35 manner.

In the embodiment shown in Fig. 1, the fused metal accumulates in the crucible and its level rises to the point of contact with the contact points 35 of a signal system 36, 40 whereupon a displacing plunger 37 of inert material of high fusion point, may be lowered into the molten metal to cause the overflow of a measured quantity of the metal for the production of pigs.

45 It will be apparent from the above example of the invention that the principles are applicable to those metals which can be reduced below the fusion point and subjected to a separation step either magnetically 50 formed as in the present example, or in some other manner which does not require slagging of the aluminous or silicaceous materials. It is also apparent that the features of the magnetic separator herein shown, are 55 applicable to the ores of magnetic metals such as iron, nickel, cobalt, etc., which can be reduced below the fusion point or which may be otherwise obtained in the form of a non-coherent mixture of finely divided metal 60 and gangue.

In place of natural gas or any gaseous reducing agent, I may employ a solid or other suitable reducing agent, as for example coal, which may be introduced with 65 the finely crushed ore into the reduction

drum. The subsequent separation step lends itself to the avoidance of the reducing agent in the purified product, as the ash would be eliminated as well as the gangue.

70 For the manufacture of steel and alloys of iron, suitable addition agents may be introduced into the pure iron crucible or the extrusion apparatus.

I claim:—

1. The method of obtaining values from 75 ores which are reducible below fusion temperature, which comprises reducing the values in finely divided ore by the incomplete combustion of hydrocarbon gas with a deficiency of air in the presence of the ore to be reduced, and separating the reduced values in finely divided solid form from the commingled gangue.

2. The method of obtaining values from 80 ores, which are reducible below fusion temperature, which comprises reducing the values in finely divided ore, without fusion, by the incomplete combustion of hydrocarbon gas with a deficiency of air in the 85 presence of the ore to be reduced, separating the reduced finely divided values from the gangue in the atmosphere of the incoming hydrocarbon gas prior to commingling of the latter with the deficiency 90 of air for combustion, and consolidating the separated values.

3. The method of obtaining values from 95 ores, which are reducible below fusion temperature, which comprises reducing the 100 values in finely divided ore, without fusion, by the incomplete combustion of hydrocarbon gas with a deficiency of air in the presence of the ore to be reduced, separating the reduced finely divided values from 105 the gangue in the atmosphere of the incoming hydrocarbon gas prior to commingling of the latter with the deficiency 110 of air for combustion, and fusing the separated values.

4. The method of obtaining values from 115 ore, which comprises reducing the values in finely divided ore to metallic state at a temperature below the fusion point of the values, separating the values from the commingled gangue while still maintaining the temperature below the fusion point, subsequently fusing the values into a coherent product, and displacing a predetermined amount of the fused metal from time to 120 time to cause the measured overflow of a unit product.

5. The method of obtaining values from 125 ore, which comprises subjecting the finely divided ore at low red heat to a reducing gas to obtain a commingled mass of finely divided non-coherent metal and gangue, separating the metal in finely divided solid form from the gangue, thereafter fusing the metal to obtain a coherent product, and dis- 130

placing a predetermined amount of the fused metal from time to time to cause the measured overflow of a unit product.

6. The method of obtaining values from 5 ore of magnetic metal, which comprises reducing the values in the finely divided ore to non-coherent metallic state, exposing the resultant mixture of finely divided materials to a magnetic flux for the separation 10 of the metal from the gangue then fusing the metal to obtain a product in coherent form, and displacing a predetermined amount of the fused metal from time to 15 time to cause the measured overflow of a unit product.

7. The method of obtaining values from ore of magnetic metal, which comprises subjecting the finely divided ore to the action of a reducing gas at a temperature below the fusion point of the metal, whereby a 20 finely divided non-coherent mixture of gangue, and metal is obtained, magnetically separating the metal from the gangue, then fusing the metal to obtain a product in coherent form, and displacing a predetermined amount of the fused metal from time to 25 time to cause the measured overflow of a unit product.

CHARLES S. BRADLEY.